

## UNITED STATES PATENT OFFICE

2,482,185

FLOOR COVERING AND COMPOSITION  
MATERIAL THEREFOR

Fred Hubert, Jr., Essex County, and Vernon A. Kildare, Bergen County, N. J., assignors to Congoleum-Nairn Inc., a corporation of New York

No Drawing. Application December 20, 1946,  
Serial No. 717,594

4 Claims. (Cl. 117—168)

1

This invention relates to floor coverings and composition material therefor, and is concerned more particularly with floor coverings of the flexible smooth surface type comprising a strain-resistant base sheet and a surface layer of wear-resistant composition material integrally united with the base sheet.

It is a purpose of this invention to provide an inexpensive floor covering made from low cost ingredients and by economical manufacturing processes which possesses good flexibility in combination with toughness and high resistance to wear and to indentation under load.

Heretofore, it has been proposed to manufacture flexible smooth surface floor coverings using as the binder for the surface layer of composition material pitch derived from animal or vegetable oils such as the pitch material which is commonly referred to as "stearin" pitch. However, such floor coverings, while having the advantage of low cost, also have the disadvantage of being deficient in flexibility with the result that the surface layer is excessively susceptible to cracking when the floor covering is subjected to flexure. Prior attempts to modify stearin pitch or the like by inclusion of minor amounts of natural or petroleum residue bitumens, have not been successful in overcoming the difficulty above mentioned.

The present invention is directed to a specific formulation of the composition material of the surface layer of a floor covering of the type in question whereby the flexibility of the composition material of the surface layer of the floor covering is much improved without impairing its hardness, wear resistance and indentation resistance.

According to this invention, the composition material for the surface layer of a floor covering of the type in question employs a mixture of cottonseed pitch and a small amount of gilsonite which mixture is modified by the presence of a small but critical amount of sulphur and is further modified by the incorporation of a calcareous filler such as powdered limestone. The composition material may likewise contain pigments or the like to provide suitable color, but the specific ingredients above mentioned in the proportions to be more particularly defined below are essential in affording the improvements of this invention.

In order to afford a better understanding of this invention and its employment in the manufacture of flexible smooth surface coverings, a typical preferred embodiment and its manufac-

ture are described below so that a specific illustrative example may be afforded.

According to the specific example to be described, the ingredients used for the preparation of the composition material of the surface layer of the floor covering are as follows, the percentages given below and elsewhere herein being percentages by weight.

|                                                    | Per cent |
|----------------------------------------------------|----------|
| 10 Cottonseed pitch (softening point 95-110° F.)   | 9        |
| 10 Cotton seed pitch (softening point 135-150° F.) | 19       |
| 15 Gilsonite                                       | 5        |
| 15 Sulphur                                         | 1        |
| 15 Manganese linoresinate                          | 1        |
| 20 Powdered limestone                              | 35       |
| 20 Red iron oxide pigment                          | 30       |

In preparing the composition material for the surface layer, the cottonseed pitch, gilsonite, sulphur, and manganese linoresinate are heated to a temperature of the order of 300° F. to 325° F. in a suitable mixer such as a Pfleiderer mixer or a steam jacketed pug mill. The powdered limestone and red oxide pigment are then incorporated and the composition is cooked for approximately three hours at the temperature mentioned, the mixer being kept in operation so as to accomplish a thorough mixing of the ingredients. During this period, the composition material becomes converted into a plastic mass. It is necessary that the composition material shall be plastic and readily workable in the mixer at temperatures around 300° F. and during the coating operation whereby it is spread as a surface layer on the base sheet of the flooring. It is also necessary that the composition material exhibit little or no flow at temperatures of the order of 155° F. to 200° F. at which the flooring is cured or seasoned.

40 After the mixing has been completed, the plastic composition is applied while still hot to the base sheet of the flooring. The base sheet of the flooring may typically be a sheet of asphalt saturated flooring felt, e. g., a 50 point (0.05 inch) dry felt which has been saturated to the extent of about 100% to 110% with asphalt having a softening point of about 160° F. The composition material can be spread on the base sheet as a coating layer in any suitable manner as by employment of a heated doctor blade. The coating layer preferably is applied so that its thickness is of the range 0.02 inch to 0.04 inch.

After the coating layer of composition material has been applied to the base sheet, the floor covering so produced is then stoved at a tem-

perature of the order of 155° F. to 200° F. (usually about 170° F.) for a period of about two to four days to season the composition material of the coating layer. During seasoning, the composition material of the coating layer develops the hardness and toughness required for providing a durable and wear-resistant surface layer for the floor covering.

The floor covering produced as above described is attractive in appearance and is very durable and serviceable. The surface coating layer of composition material is highly resistant to wear and is hard and resistant to indentation. At the same time, the coating layer of composition material is flexible. A flooring which is of such flexibility that a 2 x 8 inch sample at 77° F. can be bent at approximately the center with the felt backing on the inside through 180° of arc about a 4-inch diameter mandrel in about 5 seconds' time and at approximately a uniform speed without development of surface cracks, possesses flexibility which is adequate for practical purposes in that the covering is not susceptible to cracking of the surface layer when made up in rolls for shipment or during installation. The improved floor covering above described has substantially greater flexibility than that required to meet the test above described. Thus the floor covering which has been described hereinabove as affording a typical example of the practice of this invention has flexibility such that it can be bent about a mandrel 1 inch in diameter without development of cracks under the test conditions mentioned above. By contrast, a floor covering which is otherwise similar but which lacks the sulphur component of the composition material embodying this invention and which has been seasoned until the indentation resistance is the same, cannot be bent about a mandrel less than 6 inches in diameter without development of cracks and is considered commercially unsatisfactory because of its lack of flexibility due to the likelihood of development of highly objectionable surface cracks upon only moderate flexure.

The improvements afforded according to this invention result from the combined effects of the sulphur and powdered calcareous filler upon the cottonseed pitch and gilsonite during the heating that is incident to the mixing of the composition material and to the seasoning of the composition after its application as a coating layer. The sulphur that is employed in the composition must be present within very close limits. Thus, when 28 parts of cottonseed pitch are employed, the sulphur present should be not less than 0.5 part or greater than 3 parts by weight. If less than 0.5 part of sulphur is employed, the benefits resulting from its presence are not afforded to substantial degree. On the other hand, if more than 3 parts of sulphur are employed, the finished coating layer has undesirable permanent tackiness at ordinary temperatures, and the composition as a whole becomes too stiff for commercially satisfactory mixing and spreading as a coating layer. Moreover, the composition also develops unattractive color. It is ordinarily preferred that the sulphur be present in proportion such that for 28 parts by weight of cottonseed pitch there is present approximately 1 part by weight of sulphur.

The powdered calcareous filler that is used is preferably powdered limestone which should be present in substantial amount, namely, from 20 parts to 50 parts by weight of the powdered lime-

stone for each 28 parts by weight of the cottonseed pitch. Preferably the powdered limestone is present in amounts such that there are present from about 30 to about 40 parts by weight for 28 parts by weight of cottonseed pitch, the optimum proportion being 35 parts by weight. Since powdered limestone is the preferred calcareous filler, the claims call for powdered limestone in the relative proportions stated with the intent that if some other calcareous filler is substituted for powdered limestone such substitution would be the equivalent of the powdered limestone if the alkalinity of the calcareous filler used corresponds to the alkalinity of the stated proportions of powdered limestone. Thus, for example, if hydrated lime, which is considerably more alkaline than powdered limestone, were to be used to replace a larger proportion by weight of the powdered limestone, such substitution could be made provided the alkalinity of the resulting mixture is within the range of alkalinity afforded by the proportion range of powdered limestone stated in the claims.

Gilsonite has a softening point of about 270° to 275° F. The amount of gilsonite that is employed must be confined within narrow limits. Preferably the gilsonite should be approximately 5 parts by weight for 28 parts by weight of cottonseed pitch, the range of the gilsonite being of the order of about 4 to about 6 parts by weight for 28 parts of cottonseed pitch.

In the foregoing typical embodiment of this invention, the drier component is the drier which is commonly referred to as "manganese linoresinate" and which is a compound of the drying metal manganese with selected vegetable acids and corresponds chemically to manganese tallate (8% manganese). In addition to manganese linoresinate, other conventional driers may be employed such as manganese resinate, manganese linoleate, and manganese naphthenate. The amount of drier that is employed should be in such proportion that for 28 parts by weight of cottonseed pitch there will be present approximately 1 part by weight of drier, namely, about 0.5 part to about 2 parts by weight of the drier.

The cottonseed pitch which is the principal component of the binder for the composition material of the coating layer for the floor covering of this invention is the residue obtained from the refinement of cottonseed oil. The cottonseed pitch should have a softening point in the range from about 95° F. to about 150° F. The softening point just referred to, as well as elsewhere herein, is that determined by the standard Ring and Ball softening point test. Preferably, the softening point of the cottonseed pitch is approximately 125° F. A single cottonseed pitch may be employed or a mixture of two or more cottonseed pitches which in combination afford a cottonseed pitch mixture, the softening point of which is of the range above mentioned. It is somewhat preferable to employ a mixture consisting of one part by weight of cottonseed pitch having a softening point of about 95° F. to 110° F. and two parts by weight of cottonseed pitch having a softening point of about 135° F. to 150° F.

In addition to the foregoing essential ingredients of the composition material of the surface layer of the new floor covering of this invention, the composition material may, and ordinarily does, contain a pigment so as to impart desired color. The pigment usually employed is red iron oxide pigment, although other conventional pigments may be employed such as black iron oxide,

maroon oxide, green chromium oxide, and ochre. In addition, other finely-divided solid substantially water-insoluble filler materials may be present by way of diluents or extenders such as china clay, silica or slate flour. When it is stated that the filler is substantially water insoluble, this does not preclude the presence of a filler having slight water solubility of the order of hydrated lime.

The binder component of the composition material, namely, the cottonseed pitch, gilsonite, sulphur, and drier, preferably constitute about 30% to 35% by weight of the composition material, although the binder content of the composition material may, if desired, be varied between 30% to 65% by weight of the composition material. The balance of the composition material consists essentially of the filler including the finely-divided calcareous filler. With regard to any filler other than the calcareous filler which may be present, such other filler, for example, a pigment, should constitute from 0 to 65 parts by weight in proportion to 28 parts by weight of cottonseed pitch contained in the binder, subject, however, to the over-all limits for the relative proportions of total binder and total filler that have been stated above. Such other filler material preferably is present in such proportion as to constitute from about 25 to about 35 parts by weight in proportion to 28 parts by weight of cottonseed pitch contained in the binder, the optimum being 30 parts by weight.

When the composition material of the surface layer of the floor covering of this invention is produced within the limits of proportion and formulation stated hereinabove, the heating of the composition during mixing and during subsequent seasoning induces an interaction of the ingredients which first increases the plastic consistency of the composition and later results in the development of the tough, wear-resistant and flexible properties in the surface coating as it occurs in the finished product. In other words, in the finished product the composition material of the coating layer is the product of hardening induced by heat of the composition material that has been formulated as hereinabove described. Due to the presence of the critical proportion of sulphur, the hardening action that takes place is substantially uniform throughout the mass and improved flexibility is afforded. At the same time, the calcareous filler which is also present likewise promotes the development of the hardness of the composition material and serves to counteract the tendency of the sulphur to cause undesirable permanent tackiness of the coating layer and enables the hardness and resistance to indentation under load to be controlled without sacrifice of the flexibility afforded by the presence of the sulphur. Such action of the calcareous filler is believed to be due to its reactivity with certain acidic components of the binder material. In other words, there is an interaction of the binder ingredients with the sulphur and with the calcareous filler, which interaction results in hardening induced by heat so as to develop the hardness and indentation resistance which are required for the composition material of the surface layer of the floor covering. Notwithstanding the development of such hardness and indentation resistance the surface layer of composition material possesses greatly improved flexibility as compared with prior floor coverings of the type in question which have exhibited excessive tendency to crack upon flexure when hav-

ing sufficient hardness and indentation resistance to be useful as a floor covering. Moreover, the combination of the binder ingredients with the filler ingredients is such that the composition material can be readily and thoroughly mixed and readily spread on a base sheet as a surface layer that is excellently adapted to have its ultimate toughness and hardness developed by seasoning for only a relatively short time.

- 10 It may be mentioned that in the absence of the sulphur and calcareous filler components, a composition material otherwise similar to that above described is capable of gradual hardening when disposed as a coating layer for a floor covering by seasoning at elevated temperatures, but in such case seasoning for from 4 to 8 days at from 155° to 200° F. is required as compared with seasoning for only 2 to 4 days in the case of the composition material for the surface layer of the improved floor covering of this invention.

While this invention is ordinarily practiced by application of the composition material of the coating layer to a base sheet consisting of asphalt saturated felt, it is apparent that any other suitable strain-resisting base sheet may be employed such as burlap or other fabric or other sheet or sheet-like material. The improved floor covering of this invention can be produced in the form of a sheet of indefinite length and of any desired width or can be produced in the form of tile-like bodies. In the description of this invention and in the claims, the reference to the product as being a floor covering of the "smooth surface" type is intended to be indicative of the fact that the composition material of the surface layer has a smooth surface as distinguished from a pile fabric or the like, but is not intended to exclude the production of the surface layer so as to be embossed or so as to have differences in thickness or surface irregularities.

We claim:

1. A flexible smooth-surface floor covering comprising a flexible strain-resistant sheet-like base and a surface layer of composition material integrally united with said sheet-like base, said composition material containing from about 30% to about 65% by weight of binder and from about 35% to about 70% by weight of finely-divided substantially water-insoluble filler material and said composition material as disposed in said surface layer being the tough, flexible and wear-resistant product of the hardening induced by heat of an intimately commingled mixture consisting essentially of the following ingredients in the stated relative proportions in parts by weight:

|                                                  | Parts |
|--------------------------------------------------|-------|
| 60 Cottonseed pitch (softening point 95-150° F.) | 28    |
| Gilsonite                                        | 4-6   |
| Sulphur                                          | 0.5-3 |
| Drier for said pitch                             | 0.5-2 |
| Powdered limestone                               | 20-50 |
| 65 Filler other than said powdered limestone     | 0-65  |

2. A flexible smooth-surface floor covering comprising a flexible strain-resistant sheet-like base and a surface layer of composition material integrally united with said sheet-like base, said composition material as disposed in said surface layer of said floor covering being the tough, flexible and wear-resistant product of the hardening induced by heat of an intimately commingled mixture consisting essentially of the following in-

ingredients in approximately the stated relative proportions in parts by weight:

|                                               | Parts |
|-----------------------------------------------|-------|
| Cottonseed pitch (softening point 95-150° F.) | 28    |
| Gilsonite                                     | 5     |
| Sulphur                                       | 1     |
| Drier for said pitch                          | 1     |
| Powdered limestone                            | 30-40 |
| Filler other than said powdered limestone     | 25-35 |

3. A flexible smooth-surface floor covering comprising a base sheet of asphalt saturated felt and a surface layer of composition material integrally united with said base sheet, said composition material as disposed in said surface layer being the tough, flexible and wear-resistant product of the hardening induced by heat of an intimately commingled mixture consisting essentially of the following ingredients in approximately the proportions stated:

|                                                          | Per cent |
|----------------------------------------------------------|----------|
| Cottonseed pitch (softening point approximately 125° F.) | 28       |
| Gilsonite                                                | 5        |
| Sulphur                                                  | 1        |
| Drier for said pitch                                     | 1        |
| Powdered limestone                                       | 35       |
| Pigment                                                  | 30       |

4. A composition material adapted for application as the surface layer of a flexible smooth-surface floor covering and adapted to be hardened

upon being subjected to heat to provide a surface layer for said floor covering which is tough, flexible and wear-resistant, said composition material containing from about 30% to about 65% by weight of binder and from about 35% to about 70% by weight of finely-divided substantially water-insoluble filler material intimately commingled with said binder and said composition material consisting essentially of the following ingredients in the stated relative proportions in parts by weight:

|                                               | Parts |
|-----------------------------------------------|-------|
| Cottonseed pitch (softening point 95-150° F.) | 28    |
| Gilsonite                                     | 4-6   |
| Sulphur                                       | 0.5-3 |
| Drier for said pitch                          | 0.5-2 |
| Powdered limestone                            | 20-50 |
| Filler other than said powdered limestone     | 0-65  |

FRED HUBERT, JR.  
VERNON A. KILDARE.

#### REFERENCES CITED

The following references are of record in the file of this patent:

#### UNITED STATES PATENTS

| Number    | Name    | Date           |
|-----------|---------|----------------|
| 775,635   | Rugen   | Nov. 22, 1904  |
| 2,054,815 | Herbst  | Sept. 22, 1936 |
| 2,078,727 | Jackson | Apr. 27, 1937  |